

May 17, 1966

F. VAN LOON SHALLCROSS  
PICKUP TUBE HAVING A PHOTOCONDUCTIVE TARGET  
OF ENLARGED CRYSTAL STRUCTURE  
Filed July 6, 1962

3,252,029



Fig. 1.



Fig. 2.



Fig. 3.

INVENTOR.  
FRANK VAN LOON SHALLCROSS  
BY  
C. Lance Marshall, Jr.

ATTORNEY

1

3,252,029  
**PICKUP TUBE HAVING A PHOTOCONDUCTIVE TARGET OF ENLARGED CRYSTAL STRUCTURE**  
Frank Van Loon Shallcross, Princeton Junction, N.J., assignor to Radio Corporation of America, a corporation of Delaware

Filed July 6, 1962, Ser. No. 207,993  
6 Claims. (Cl. 313—65)

This invention relates to photosensitive devices. In particular, this invention relates to novel photoconductive type pickup tubes.

In the prior art there is a commercially available photoconductive pickup tube, or device, which is known as the vidicon. The vidicon normally includes an evacuated envelope having an electron gun in one end thereof. In the other end of the envelope there is a transparent electrically conducting signal plate on which is deposited a layer of photoconductive material. When an image is focussed onto the photoconductive material, a charge is developed on the beam side of the photoconductive material which is then read off by the electron beam to provide output signals from the signal plate of the tube.

Tubes of the type briefly described above are limited by the gain obtainable from the photoconductor and by the response time of the photoconductor. Thus, the sensitivity of the tube is controlled primarily by the gain obtainable from the layer of photoconductive material. The speed of response is controlled partly by the circuits used, and partially by the time which elapses between when the image strikes the photoconductor and when the charge is developed on the beam side of the photoconductor. The speed of response is also affected by the time required for the beam to remove the charge produced by the light after the light image has been removed.

It is therefore an object of this invention to provide a new and novel pickup or camera tube.

It is another object of this invention to provide an improved camera tube having a novel photoconductive layer characterized in its high quantum gain and short response time.

These and other objects are accomplished in accordance with this invention by providing a pickup or camera tube having a recrystallized photoconductive target electrode in which the crystals of photoconductive material are large, i.e., the crystallites are at least as large as the film thickness. The crystallite size is preferably selected so that grain boundaries cannot be resolved by the beam. The visibility of the grain boundaries in the transmitted picture can also be avoided by forming the entire target area of a single crystal.

The invention will be more clearly understood by reference to the accompanying single sheet of drawings wherein:

FIG. 1 is a sectional view of a pickup tube made in accordance with this invention;

FIG. 2 is an enlarged sectional view of the target during a stage of manufacturing, for use in the tube illustrated in FIG. 1; and,

FIG. 3 is an enlarged sectional view of a target shown in FIG. 1.

Referring now to FIG. 1 in detail, there is shown a photoconductive type pickup tube 10. The pickup tube 10 is an example of a tube wherein this invention is particularly useful, and the invention will be explained in detail in connection with this type of tube. The tube 10 comprises an evacuated envelope 12 having an electron gun assembly 14 positioned in one end thereof for producing an electron beam. By means of potentials applied to the electron gun 14 and to an accelerating electrode 16,

2

as well as by means of appropriate magnetic fields from conventional alignment coils, focus coils and a deflection yoke (none of which are shown for simplicity of illustration) the electron beam is directed toward and scanned over a photoconductive target electrode 18. It should be understood that electrostatic deflection and focussing could be used in place of the magnetic system described.

The target electrode 18, which is shown more clearly in FIG. 3, comprises a transparent electrically conductive electrode 20 deposited on a transparent face plate 22. The face plate 22 forms an end of the envelope 12. The transparent electrically conductive electrode 20 is made of a material that is selected for its transparency to radiations of the particular wavelengths of interest and for its electrical conductivity. For the visible range of wavelengths, a layer of tin oxide is conventionally used. The transparent conductive coating 20 is deposited in contact with an electrically conductive sealing ring 24 so that, during operation of the device 10, an electrical potential may be applied to the transparent conductive electrode 20 and the transparent conductive electrode may function as a signal plate for obtaining output signals from the device 10.

On the transparent conductive electrode 20 there is deposited a layer of photoconductive material 26. The photoconductive material 26 comprises large area crystals rather than microcrystalline or amorphous films. The large area crystals are used because of the high quantum gains obtainable from such a film and the short response times that have been observed in such films. Specifically, the photoconductive material 26 is single-crystalline, i.e., one crystal is used which is at least the size of the scanned raster, to a maximum dimension substantially equal to the vidicon target shown in FIG. 1, or polycrystalline with the crystallites being at least as large as the film thickness. Film thickness within the approximate range of two to ten microns are conventionally used. Thus, targets for the tube of FIG. 1 are primarily composed of crystallites varying in size from a minimum size having at least one dimension that is at least as large as the film thickness to a maximum size of one crystal per tube. Within this range, the crystallite size is preferably selected so that the grain boundaries cannot be resolved by the beam. Thus, a single crystal is a preferred size since the grain boundaries would not be resolved by the beam. Also, crystallites of a size approximately equal to the beam resolving power, i.e. conventionally 10 to 100 microns, cannot be resolved by the beam and are also a preferred size.

The deposition of the photoconductive layer 26, illustrated in FIG. 2, is by means of a recrystallized photoconductive layer. By recrystallization is meant the process wherein a photoconductive material is deposited, usually by evaporation, onto the target. The deposited layer may or may not include crystals. Subsequently, the deposited layer is processed to form large crystals. As was previously stated the crystals so formed by the recrystallization process have at least one dimension that is at least as large as the film thickness. For example, a polycrystalline cadmium sulfide film has been coated on a tin oxide electrically conducting electrode 20 by vacuum evaporating cadmium sulfide material on top of the electrode 20 with a substrate temperature of about 170° C. The impurities present will mainly be lost during the evaporation process. Therefore, impurity levels of a few hundred parts per million may be used. The evaporation is continued until cadmium sulfide material is deposited to a thickness of about 4 microns. The cadmium sulfide film was then baked at atmospheric pressure in an atmosphere of air and sulfur vapor with a sulfur

vapor pressure of approximately one to ten mm. Hg, and at a temperature of 250° C. to 260° C. for approximately three hours. A layer of silver 27 was then evaporated onto the photoconductive material (the cadmium sulfide) to a thickness of approximately 120 Angstrom units. The target 18 was then heated in argon at atmospheric pressure to a temperature of approximately 520° C. for a period of time of approximately one hour to recrystallize the cadmium sulfide. On subsequent examination of a film, manufactured as described above, it was seen that the photoconductor was recrystallized with crystallites of approximately 1 mm. dimensions.

Another method of forming a recrystallized cadmium sulfide layer is by first evaporating a layer of silver, then the cadmium sulfide material rather than the opposite order as was described above. This latter method will minimize the problem of a high surface conductivity layer, or spots of silver, affecting resolution of the stored image in the completed target.

Materials other than silver, examples of which are copper and indium or mixtures thereof, may also be used to promote recrystallization of cadmium sulfide and may be deposited either under or over the cadmium sulfide material.

Other photoconductive materials may also be prepared in the form of single crystals, or large crystals, having crystallite sizes that have at least one dimension that is at least as large as the film thickness. Known photoconductive materials which are believed to be capable of being formed in this crystal size by a recrystallization process include cadmium selenide, zinc selenide, zinc sulfide, arsenic trisulfide, antimony trisulfide, cadmium-indium sulfide, and zinc-indium sulfide.

In FIG. 3 there is illustrated schematically a sectional view of a recrystallized layer of photoconductive material 26 deposited on the transparent signal plate 20. As illustrated there are a plurality of crystallites included in the target 18. The target area is substantially covered by crystallites which have at least one dimension that is within the range of being at least as large as the film thickness up to a maximum size of a single crystal over the complete target. As was previously stated, within this range, the crystallites are preferably of such a size that the grain boundaries cannot be resolved by the beam.

The very high gain materials described in this invention may also be prepared having lower resistivities than those used in the prior art tubes. Thus, depending upon the material selected and its intended use, these materials may have a sufficiently high gain that conventional charge storage is not necessary for operation. Thus, in this latter type of operation those photons striking a given elemental area during the interval between scans increase the conductivity of the photoconductor in this area, thus affecting the size of the current pulse which flows in the photoconductor at the instant of scanning. As is obvious, extremely high gains would be necessary in this mode of operation since some photoexcited charge is lost by recombination between scans.

Thus, this invention describes a recrystallized film of photoconductive material in which the crystallites are at least as large as the film thickness. By means of this invention, much higher quantum gains with short response time may be obtained which are much greater than those obtainable with conventional photoconductors now used in the vidicon. The use of such materials in the vidicon are believed to provide higher sensitivity with improved response times in the charge-storage mode of operation as well as permitting other types of operation not requiring charge storage. It should be clearly understood that the large-crystalline films may be made sensitive to visible light as well as X-ray, ultra-violet or infrared radiation. Any desired exciting radiations may be used by selecting the spectral sensitivity range of the photoconductive materials.

I claim:

1. A pickup tube comprising an evacuated envelope:
  - (a) an electron gun in one end of said envelope for producing an electron beam;
  - (b) a target electrode in said envelope and in the path of said electron beam;
  - (c) said target electrode comprising a transparent electrode having a recrystallized layer of photoconductive material thereon;
  - (d) said recrystallized layer of photoconductive material comprising at least one crystal of photoconductor; and,
  - (e) said at least one crystal having at least one dimension that is at least as large as the thickness of said layer of photoconductive material.
2. A pickup tube as in claim 1 wherein said at least one dimension of said at least one crystal is substantially as large in width as said transparent electrode.
3. A pickup tube comprising an evacuated envelope:
  - (a) an electron gun in one end of said envelope for producing an electron beam;
  - (b) a target electrode in said envelope and in the path of said electron beam;
  - (c) means for scanning said beam in a raster over said target electrode;
  - (d) said target electrode comprising a transparent electrode having a recrystallized layer of photoconductive material thereon;
  - (e) said recrystallized layer of photoconductive material comprising at least one crystal of photoconductor; and,
  - (f) said at least one crystal being at least as large as said raster.
4. A camera tube comprising an evacuated envelope:
  - (a) an electron gun in one end of said envelope for producing an electron beam;
  - (b) a target electrode in said envelope and in the path of said electron beam;
  - (c) said target electrode comprising a transparent electrode having a recrystallized layer of photoconductive material thereon;
  - (d) said recrystallized layer of photoconductive material comprising a plurality of crystals of photoconductor;
  - (e) each of said crystals being at least as large as the thickness of said layer of photoconductive material; and,
  - (f) each of said crystals being substantially as large as the diameter of said beam.
5. A pickup tube comprising an evacuated envelope:
  - (a) an electron gun in one end of said envelope for producing an electron beam;
  - (b) a target electrode in said envelope and in the path of said electron beam;
  - (c) said target electrode comprising a transparent electrode having at least one recrystallized layer of photoconductive material thereon;
  - (d) said recrystallized layer of photoconductive material comprising at least one crystal of photoconductor;
  - (e) said at least one crystal of photoconductor having at least one dimension at least as large as the thickness of said layer of photoconductive material; and,
  - (f) said photoconductive material being selected from the group consisting of cadmium sulfide, cadmium selenide, zinc sulfide, arsenic trisulfide, antimony trisulfide, cadmium-indium sulfide, and zinc-indium sulfide.
6. A pickup tube comprising an evacuated envelope:
  - (a) an electron gun in one end of said envelope for producing an electron beam;
  - (b) a target electrode in said envelope and in the path of said electron beam;

- (c) said target electrode comprising a transparent electrode having a recrystallized layer of cadmium sulfide photoconductive material thereon;
- (d) said recrystallized layer of cadmium sulfide photoconductive material comprising at least one crystal of cadmium sulfide; and,
- (e) said at least one crystal of cadmium sulfide having at least one dimension that is at least as large as the thickness of said layer of cadmium sulfide photoconductive material.

## References Cited by the Examiner

## UNITED STATES PATENTS

3,106,488 10/1963 Lubszynski ----- 313—65 X

5 ROBERT SEGAL, *Primary Examiner.*DAVID J. GALVIN, *Examiner.*V. LAFRANCHI, *Assistant Examiner.*